

M. REES.

PROCESS OF BLUING IRON OR STEEL ARTICLES.  
APPLICATION FILED JUNE 2, 1909.

949,500.

Patented Feb. 15, 1910.



WITNESSES:

John Linn  
Agnes E. Skinker

INVENTOR:

Morgan Rees,  
by his attorney,  
Wm A. Skinker

# UNITED STATES PATENT OFFICE.

MORGAN REES, OF FOLLANSBEE, WEST VIRGINIA, ASSIGNOR OF ONE-THIRD TO  
WILLIAM A. SKINKLE, OF CLEVELAND, OHIO, AND ONE-THIRD TO WILLIAM  
THOMAS, OF PITTSBURG, PENNSYLVANIA.

## PROCESS OF BLUING IRON OR STEEL ARTICLES.

949,500.

Specification of Letters Patent. Patented Feb. 15, 1910.

Application filed June 2, 1909. Serial No. 499,710.

To all whom it may concern:

Be it known that I, MORGAN REES, a British subject, but about to become a citizen of the United States, residing at Follansbee, 5 Brooke county, West Virginia, have invented certain new and useful Improvements in Processes for Bluuing Iron and Steel Articles, of which the following is a specification, that will enable those skilled in the art to 10 which the invention pertains to practice the same, reference being had to the accompanying drawing, which forms a part hereof.

This invention relates to an improved process for bluing articles of iron or steel, 15 whereby the same attain a deep blue color, and it is particularly applicable to sheets or plates of such metals which, when polished by cold rolling or otherwise, become similar to what is known in commerce as "Russian 20 sheet iron."

For a full understanding of the invention and the merits thereof, reference is to be had to the accompanying drawing, which is a vertical section through one form of device 25 for carrying on the bluing process.

This drawing shows a form of apparatus that is now considered desirable, but obviously, many changes, not requiring the exercise of invention, might be made in the 30 details thereof by a skilful mechanic, without materially changing the essential features of the process and without departure from the spirit of the invention as set forth in the claims at the end of this specification.

To put the invention into practice, by a 35 method which has been followed with success in the bluing of sheets, for which it is particularly designed, the sheets or plates of iron or steel, as taken from the rolls or hammers, are first pickled in a mixture of sulfuric acid and other ingredients in the manner well known in the art, to remove the scale. After being thus pickled the plates are, preferably, annealed by piling them one 40 upon the other on an annealing box bottom 1, a metal cover 2, being placed upon the bottom 1, to inclose the plates, the whole then placed in an annealing furnace and heated to a high temperature, say about 1600 45 to 1800 degrees, Fahrenheit. The box and contents are removed from the furnace and allowed to stand for several hours and cool down gradually to about 600 to 700 degrees, 50 Fahrenheit.

It is important that the temperature be lowered to about this condition as it is the temperature which has been found best suited to promote the desired action of the particular gases and the steam in the bluing process herein described. A much higher temperature than 700 degrees would probably be destructive to these gases before they would have time to circulate through the pile of plates and perform their coloring functions, while a much lower temperature than 600 65 degrees would not be sufficient to properly vaporize the chemicals.

In common practice the annealing box bottom and cover are heavy, rough iron castings and the joint between them is unfinished and rough. As this joint is not tight it is customary to form a seal 3 of fine dry sand, piled several inches deep all around the joint, which seal, while not absolutely tight against the forced passage of air or 70 gas under pressure, is enough to prevent the passage of air or gas under normal atmosphere and to sufficiently protect the enclosed plates against undesirable exposure.

The annealing box 2 is fitted with steam 75 connection pipe and valve 5, which may be located at any convenient point, and the pipe is connected by a suitable coupling 6 and pipe 7 to a convenient form of device 80 for introducing the chemicals, in powdered form, into the interior of the annealing box 2 in conjunction with the steam. The chemicals, which are thus carried into the annealing box by the steam passing through connection 5 are sulfur and charcoal or carbon, preferably, in powdered form, in about equal proportions, from three to four ounces of them being used to four to five tons of 85 steel or iron plates.

The device for holding the chemicals, 90 which may be mixed, if desired, to form a powdered composition, consists of a box 8 having a steam inlet pipe 9 entering the same, the said pipe being formed with a jet opening 10 arranged opposite to the 100 opening 11 leading to the pipe 7, so that the ingredients placed in the upper compartment 12 of the device will be gradually fed down into the path of the steam jet and be forced along with the steam or moisture into 105 the annealing box 2. In the construction shown on the drawing the compartment 12 is formed with a perforated bottom 14 and

a perforated plate 13 rests upon the bottom and co-operates therewith to regulate the quantity of the ingredients which are dropped upon the inclined plate 15 beneath the bottom. A lid or cover 16 is provided for closing the compartment, and the ingredients which drop through the perforated bottom of the compartment upon the inclined plate 15 are carried by the steam 10 into the interior of the annealing box so as to act upon the plates therein.

Steam alone may be let into the annealing box by way of the pipe 17.

When the annealing box is closed over 15 the pile of plates the considerable unoccupied spaces are filled with air, which, when subjected to the heat of the annealing, expands and causes a slight pressure under which some of the air will escape by seeping out through the sand seal. When the box, after withdrawal from the annealing 20 furnace, is cooling down the remaining air in it will contract and thus create a slight vacuum, to relieve which some outside air 25 will seep back, through the hot sand seal, into the box.

Another method of using the powdered ingredients is to remove from several places or spots the sand forming the seal 3 between 30 the bottom 1 and the box 2 and to place the powder in these bared spaces close against the side of the cover and adjacent to the joint opening, then return the hot sand upon 35 the top of the powder, and moisten the sand with water. The powdered sulfur and carbon thus placed will be converted into gases and the water into steam by their hot environment, and these will be drawn into the 40 box through the joint by reason of the vacuum caused by the continued cooling and contraction of the air within. The gases and steam thus find their way into the box where there is already a quantity of air with which 45 they commingle and circulate around and through the pile of plates. A jet of live steam may also be used at this juncture with good effect to give additional moisture to the gaseous mixture and to agitate and 50 quicken it into more active circulation about and through the plates. The sulfur and carbon are used in powdered form only for the convenience of the operator in handling them with this form of apparatus, but it 55 will be obvious that immediately upon their entrance into the box they meet with the heated air already in the box or come into contact with the heated metal of the box or with the pile of heated plates therein and 60 are at once converted into gases, which together with the steam attack the surfaces of the plates and give them a deep blue color. It will be understood, therefore, that 65 it is the hot sulfur and carbon gases together with the moisture of the steam and the hot air already in the box that do the bluing

of the plates; and that with suitable apparatus the sulfur and carbon might be vaporized previously to their introduction into the box. This is considered to be within the limits of the invention. These gases may be 70 introduced either separately or together, and either before or together with the steam. If the gases are applied separately it is considered preferable to use the sulfur first, then the carbon and later, after an interval 75 of say ten to thirty minutes, the steam. It has been found however that considerable latitude may be had in this respect without materially affecting the result and that no very hard and fast rule need be followed. 80

After the introduction of sufficient chemicals, or their gases, and the steam the box is allowed to remain closed for a number of hours until it and the plates within it have cooled down slowly to about the normal 85 temperature of the outer air, when the bluing process is finished.

The sheets, when taken from the box will have a deep blue color over their entire surfaces, and should it be desired to polish 90 the plates, the cold rolling process is used in the manner well known in the art.

Care should be taken that the box be kept closed and the plates not exposed to the cold outside air at any stage of the process and 95 that no outer air be admitted to the box except, perhaps, such small quantity as may seep or be drawn in through the seal of hot sand during the cooling down period.

In the foregoing I have described the 100 process as practiced with an annealing box, and this will, doubtless, be the most usual manner of practicing it as most plate-finishing mills anneal their plates and are, therefore, already provided with suitable boxes. 105 Pre-annealing, however, is not essential for the practice of this invention, and the bluing may be carried on in any suitable closed vessel, oven, chamber or receptacle in which the plates may be heated without exposure 110 to the direct action of the furnace fire. It has also been described that the plates are first subjected to the high temperature, 1600 to 1800 degrees Fahrenheit, necessary in the annealing process, but cold and un-annealed 115 plates may be blued by simply heating them in a closed receptacle up to about 650 degrees, Fahrenheit, which has been found to be about right for this process of bluing.

Pickling, to remove the scale and other impurities from the surfaces of the plates, while not a step in this invention, is quite necessary for the production of finely finished plates and it should always be done before the bluing process for finished work. 120

While the process has been described, herein, in its application to bluing iron and steel plates or sheets, it is not meant to limit its use to these forms for, as will be readily understood, it is equally applicable to blu- 125 130

ing the surfaces of other forms of iron or steel articles.

Having thus described the invention, what is claimed as new is:—

- 5 1. The process of bluing iron or steel articles which consists of placing said articles in a closed receptacle, heating and subjecting them to the action of sulfur and carbon gases together with steam and the heated air already in the receptacle.
- 10 2. The process of bluing iron or steel articles which consists of placing said articles in a closed receptacle and heating them to about 650 degrees, Fahrenheit, and then subjecting them to the action of sulfur and carbon gases together with steam and the heated air already in the receptacle.
- 15 3. The process of bluing iron or steel articles which consists of placing them in a closed receptacle and heating them to about 650 degrees, Fahrenheit, then injecting first sulfur and carbon gases into the receptacle and later a jet of steam.
- 20 4. The process of bluing iron or steel articles which consists of placing them in a closed receptacle, heating them and subjecting them to the action of sulfur and carbon gases and steam together with the heated air already in the receptacle and then allowing them to cool in the closed receptacle. 30

In testimony whereof I have signed my name to this specification in the presence of two subscribing witnesses.

MORGAN REES.

Witnesses:

TREVOR THOMAS.  
ALBERT JAMES.